

# United States Patent

Leung

[15] 3,652,199

[45] Mar. 28, 1972

[54] **PROCESS FOR DRYING POLYAMIDE FIBERS CATIONIC DYES AND ZINC THIOCYANATE**

[72] Inventor: Peter S. K. Leung, Wilmington, Del.

[73] Assignee: E. I. du Pont de Nemours and Company, Wilmington, Del.

[22] Filed: Aug. 28, 1969

[21] Appl. No.: 853,924

[52] U.S. Cl.....8/30, 8/178

[51] Int. Cl. ....D06p 3/24

[58] Field of Search .....8/178 R, 175, 172, 166, 177 AB,  
8/99, 30; 260/78

[56] **References Cited**

## UNITED STATES PATENTS

|           |         |               |                |
|-----------|---------|---------------|----------------|
| 3,063,966 | 11/1962 | Kwolek et al. | .....260/78    |
| 3,338,660 | 8/1967  | Biederman     | .....8/178 R X |
| 3,349,062 | 10/1967 | Hill et al.   | .....8/178 R X |

3,506,990 4/1970 Richardson et al. ....8/172

## FOREIGN PATENTS OR APPLICATIONS

|         |        |                     |         |
|---------|--------|---------------------|---------|
| 794,753 | 9/1968 | Canada .....        | 8/178 R |
| 603,154 | 6/1948 | Great Britain ..... | 8/178 R |
| 642,840 | 9/1950 | Great Britain ..... | 8/175   |
| 813,289 | 5/1959 | Great Britain ..... | 8/175   |

## OTHER PUBLICATIONS

R. W. Schumm et al.,



(A publication by

AATCC), Aug. 27, 1969, Vol. 1, No. 18, pages 27-30

Primary Examiner—Donald Levy

Assistant Examiner—T. J. Herbert, Jr.

Attorney—John E. Dull

[57]

## ABSTRACT

Process for dyeing polyamide fibers with a cationic dye comprising treating said fibers with an aqueous bath containing a cationic dye and zinc thiocyanate at a temperature of at least 90° C.

**5 Claims, No Drawings**

**PROCESS FOR DRYING POLYAMIDE FIBERS CATIONIC DYES AND ZINC THIOLYANATE**

**BACKGROUND OF THE INVENTION**

This invention concerns a process for dyeing polyamide fibers with cationic dyes. These dyes are of particular interest for use in polyamides because of their bright shades, particularly in the red and pink colors and because of the fluorescence which some of the cationic dyes display.

Polyamide fibers have been the subject of much research in the field of dyeing, and numerous dyes are available, particularly in the disperse dye and acid dye categories. However, the cationic dyes have been characterized by poor affinity and poor wash fasteners when applied to polyamide fibers. Fibers of polyamides containing aromatic or cyclohexane constituents are especially resistant to cationic dyes.

**SUMMARY OF THE INVENTION**

The present invention provides a process for dyeing polyamide fibers with a cationic dye comprising contacting said fibers with an aqueous bath containing a cationic dye and zinc thiocyanate at a temperature of at least 90° C., the amount of zinc thiocyanate in the bath being from 1 to 60 percent based on the weight of said fibers and less than 1.5 percent based on the weight of water in the bath. This invention provides a process whereby cationic dyes can be applied to polyamide fibers in much the same manner as disperse dyes, i.e. by dissolving in the fiber and diffusing through it. The process is particularly useful for the polyamides containing aromatic constituents or cyclohexane constituents.

**DESCRIPTION OF THE PREFERRED EMBODIMENTS**

The polyamide fibers which may be dyed by the process of this invention include all of the commonly known polyamides such as poly(hexamethylene adipamide), the polymers obtained from  $\xi$ -caprolactam, and copolymers of these. The process is particularly useful for application of cationic dyes to fibers of polyamides containing aromatic constituents, such as disclosed in U.S. Pat. No. 3,063,966, and polyamides containing cyclohexane constituents, such as disclosed in U.S. Pat. No. 3,393,210. The preferred polyamides are poly(meta-phenylene isophthalamide) and the polymer derived from bis(4-aminocyclohexyl)-methane and dodecanedioic acid, i.e., poly(methylene-di-1,4-cyclohexylene dodecane diamide).

The cationic dyes (sometimes known as basic dyes), in general, are chemical mixtures containing compounds with one or more onium groups such as the quaternary ammonium group. The onium groups carry a positive charge; hence the name "cationic." The principal constituent may also contain some anionic water-solubilizing groups such as sulfonic or carboxylic acid groups provided that there are more equivalents of the cationic groups than of the anionic groups. A large number of suitable cationic dyes is disclosed in Canadian Pat. No. 794,953. Other useful cationic dyes are disclosed in U.S. Pat. No. 3,338,660.

The aqueous dye bath used in this invention must contain zinc thiocyanate which promotes high color yield and high wash fastness without affecting appreciably the physical properties of the fiber. The color yield for cationic dyes applied to polyamide fibers in the presence of zinc thiocyanate is usually at least 2.5 times as great as the color yield without zinc thiocyanate. The color yield of the dyed fibrous polyamides is measured by the K/S value (Kubelka-Munk absorption-scattering factor) which is calculated from the expression

$$K/S = (1-R)^2/2R$$

where R is the fraction of light reflected at maximum absorption wavelength from the dyed yarn or fabric. To obtain a relative color yield the K/S value for dyeing in the presence of the anionic agent is divided by the K/S value obtained in the absence of the anionic agent and multiplied by 100. In the process of the invention, the dye bath may contain zinc thiocyanate or its equivalent ionic components. It should be understood that the zinc cations, thiocyanate anions, or thiocyanate complex ions may be supplied from separate chemicals. It is only essential that the zinc cation and thiocyanate anion be available in sufficient quantity to give 1 to 60 percent of the equivalent zinc thiocyanate based on the weight of the fibers and less than 1.5 percent by weight based on weight of water in the bath.

5 Analysis of polyamide yarns after dyeing indicates that zinc and sulfur atoms are present in a 1:4 ratio. This ratio seems to indicate that a complex is formed between the zinc thiocyanate and the dye molecule, the composition being perhaps, [Dye<sup>+</sup>]<sub>2</sub>[Zn(SCN)<sub>4</sub>]. Therefore, the zinc ion and the thiocyanate ion are no longer present in the 1:2 ratio of Zn(SCN)<sub>2</sub>. The 1:4 ratio is maintained regardless of dye concentration. The dye complex may possibly act through a disperse dyeing mechanism. The ratio by weight of zinc thiocyanate to the dye weight is not critical, and in fact the optimum thiocyanate concentration in the bath may be considerably more than would be required to provide one equivalent of zinc for one equivalent of dye. It is believed that the additional zinc thiocyanate acts as a swelling agent for the fiber and for the dye complex thereby promoting diffusion.

10 It is surprising to note that other thiocyanates are relatively inferior in promoting the dyeing of polyamides with cationic dyes. The superiority of zinc thiocyanate is not completely understood, but it is definitely superior to other thiocyanates.

15 While the aqueous dye bath need not contain any additional dye carriers, it is often desirable to use such dye carriers when difficultly dyeable polyamide fibers are being processed. In particular, dye carriers are useful in dyeing poly(meta-phenylene isophthalamide) fibers and poly-(methylene-di-1,4-cyclohexylene dodecane diamide) fibers. Suitable dye carriers for these two types of fibers include butyl benzoate, pelargonic acid, mixtures of benzaldehyde and dimethyl terephthalate, o-phenyl phenol, chlorinated benzene, biphenyl, and methyl salicylate.

20 In the practice of this invention, the temperature of the aqueous dye bath is at least 194°F. (90°C.), but usually less than about 270°F. (132°C.). Obviously, adequate pressure equipment must be provided for dyeing in aqueous baths at temperatures above 212°F. (100°C.).

25 In this invention, the aqueous dye bath preferably is acidic. Conventional dye bath additives also may be used, if desired, such as surface active agents and leveling agents. Citric acid is a particularly desirable leveling agent.

30 The following examples further illustrate preferred embodiments of this invention. In these examples, poly(meta-phenylene isophthalamide) is abbreviated "MPD-I" and poly-(methylene-di-1,4-cyclohexylene dodecane diamide) is abbreviated "PACM-12." In these examples, all percentages are on a weight basis.

**EXAMPLE I**

**55 EFFECT OF ZINC THIOLYANATE CONCENTRATION ON COLOR VALUE FOR MPD-I SAMPLES**

60 Ten swatches of fabric woven from MPD-I fibers weighing 10 g. each are introduced into 10 separate aqueous baths at 100°F. (38°C.). Each bath contains 0.1 G. "Merpol" HCS (a nonionic surfactant), 1.5 gm. "Latyl" Carrier A (a mixture of benzaldehyde and dimethyl terephthalate), 4 g. glacial acetic acid, 0.3 g. "Calcozine" Acrylic Blue HP (a cationic dye, Color Index Basic Blue 54). Each bath contains a different amount of zinc thiocyanate as indicated in Table 1. The baths containing the fabric samples are heated to 250°F. (121°C.) and kept at this temperature for 2 hours. After this the samples are removed from the baths and rinsed. Then the dyed samples are scoured for 30 minutes in 400 ml. of aqueous bath 65 containing 0.1 g. "Merpol" HCS (nonionic surfactant) and 0.1 g. tetrasodium pyrophosphate at a temperature of 200°F. (93°C.). The dyed and scoured material is then rinsed and dried. A series of blue dyed fabric samples are obtained which have good wash fastness. The color yield for each of the dyes is indicated in Table 1.

TABLE 1

| % Zinc Thiocyanate |                |                |           |                      |
|--------------------|----------------|----------------|-----------|----------------------|
| Bath               | Based on Water | Based on Fiber | K/S Value | Relative Color Yield |
| 1                  | 0              | 0              | 0.88      | 100                  |
| 2                  | 0.125          | 5              | 2.24      | 254                  |
| 3                  | 0.250          | 10             | 2.45      | 279                  |
| 4                  | 0.375          | 15             | 2.20      | 250                  |
| 5                  | 0.500          | 20             | 2.20      | 250                  |
| 6                  | 0.625          | 25             | 1.22      | 138                  |
| 7                  | 0.750          | 30             | 1.71      | 195                  |
| 8                  | 0.875          | 35             | 1.55      | 176                  |
| 9                  | 1.000          | 40             | 1.67      | 189                  |
| 10                 | 1.25           | 45             | 1.59      | 181                  |

## EXAMPLE II

## EFFECT OF ZINC THIOCYANATE CONCENTRATION ON CATIONIC DYEING OF PACM-12

Twenty-one swatches of fabric woven from PACM-12 fibers, each weighing 5 g., are introduced into 21 separate 200 ml. warm baths (38°C.). Seven of the baths contain 0.1 g. "Astrazon" Yellow 7GLL (a cationic dye, Color Index Basic Yellow 21). Seven others contain 0.1 g. "Sevron" Brilliant Red D (a cationic dye, Color Index Basic Red 19). Another seven contain 0.1 g. "Sevron" Blue EG (a cationic dye, Color Index Basic Blue). Each of the baths also contains 4 g. citric acid, 0.05 g. "Merpel" HCS, 0.75 g. "Cindy" DAC 888 (butyl benzoate) and zinc thiocyanate as indicated in Table 2. The baths are heated to 212°F. (100°C.) and kept at this temperature for 90 minutes. The dyed swatches are then removed from the dye bath and rinsed. Then they are scoured for 30 minutes at 180°F. (82°C.) in 200 ml. aqueous baths containing 0.05 g. "Merpel" HCS and 0.05 g. tetrasodium pyrophosphate. The swatches are then rinsed and dried. A series of yellow, red, and blue dyeings are obtained which have good wash fastness.

The effect of zinc thiocyanate concentration on color yield as measured by the K/S value is indicated in Table 2.

TABLE 2

| % Zinc Thiocyanate |                |                |           |                   |            |
|--------------------|----------------|----------------|-----------|-------------------|------------|
| Bath               | Based on Water | Based on Fiber | Yellow 21 | K/S Values Red 19 | Basic Blue |
| 1                  | 0              | 0              | 0.35      | 2.07              | 2.55       |
| 2                  | 0.25           | 10             | 2.65      | 3.55              | 5.16       |
| 3                  | 0.50           | 20             | 4.15      | 4.98              | 6.65       |
| 4                  | 0.75           | 30             | 4.87      | 5.60              | 6.92       |
| 5                  | 1.00           | 40             | 5.06      | 6.13              | 7.25       |
| 6                  | 1.25           | 50             | 5.08      | 6.60              | 7.65       |
| 7                  | 1.50           | 60             | 5.12      | 5.92              | 7.65       |

## EXAMPLE III

## EFFECT OF VARIOUS DYE CARRIERS ON CATIONIC DYEING MPD-I

Ten swatches (10 g.) of MPD-I woven fabric are introduced into 10 separate aqueous baths at 100°F. (38°C.) each containing 0.1 g. "Merpel" HCS, 4 g. glacial acetic acid, 4.0 g. zinc thiocyanate (1 percent based on water, 25 percent based on fiber), 0.3 g. "Calcozine" Acrylic Blue HP (Color Index Basic Blue 54) and 1.5 g. of a dye carrier. Several separate dyeings were run, each with a different dye carrier. The effects of various dye carriers on color yield measured by the K/S

70

value are listed in Table 3. The carriers were added in sufficient quantity to give 15 percent by weight, based on fiber. The 10 baths each containing a different carrier or no carrier were heated to 250°F. (121°C.) and kept at this temperature for 2 hours. The dyed materials were then removed from each of the dye baths and rinsed. Then the dyed materials were scoured for 30 minutes in 400 ml. of another aqueous bath containing 0.1 g. "Merpel" HCS and 0.1 g. tetrasodium pyrophosphate at a temperature of 200°F. (93°C.). The dyed and scoured materials were then rinsed and dried. A series of blue dyeings is obtained which have good wash fastness.

TABLE 3

| 15 | Dye Carrier                                       | Color Yield K/S |
|----|---------------------------------------------------|-----------------|
| 20 | None                                              | 1.154           |
|    | "Phenetol" D                                      | 1.600           |
|    | Mixture of emulsified organic solvents            | 1.713           |
|    | "Cindy" DAC-888                                   |                 |
|    | Butyl benzoate                                    |                 |
|    | Pelargonic Acid                                   | 1.542           |
|    | "Laty" Carrier A                                  | 1.883           |
|    | Mixture of benzanilide and dimethyl terephthalate |                 |
|    | "Carolid" 50                                      | 2.010           |
|    | o-Phenylphenol                                    |                 |
|    | "Chemo" Carrier KDSW                              | 1.179           |
|    | Dimethyl phthalate                                |                 |
|    | "Tanavol"                                         | 1.646           |
|    | Chlorinated benzene                               |                 |
|    | "Charlab" M-1                                     | 1.613           |
|    | Biphenyl                                          |                 |
|    | Methyl salicylate                                 | 1.624           |

## EXAMPLE IV

## EFFECT OF VARIOUS DYE CARRIERS ON CATIONIC DYEING OF FABRICS OF PACM-12

40 Swatches (5 g.) of PACM-12 woven fabric are introduced into 51 separate aqueous baths at 100°F. (38°C.). Each of the baths contains 200 ml. of water, 4 g. citric acid, 0.05 g. "Merpel" HCS, 2 g. zinc thiocyanate (1 percent based on water, 40 percent based on fiber), and 0.75 g. of one of the dye carriers shown in Table 4. In addition, one of the three dyes shown in Table 4 is added. In each case the amount of dye is 0.1 g. The bath is then heated to 212°F. (100°C.) and kept at this temperature for 90 minutes. The dyed fabric samples are then removed from the dye baths and rinsed. Then, the dyed samples are scoured for 30 minutes at 180°F. (82°C.) in 200 ml. of another aqueous bath containing 0.05 g. "Merpel" HCS and 0.05 g. tetrasodium pyrophosphate. The dyed and scoured materials are then rinsed and dried. A series of orange, red and blue dyeings are obtained which have good wash fastness.

45 The effect of various dye carriers on color yield is determined by measurement of K/S values for the dyed fabrics. Fabrics which were dyed in the same way but without carrier were also measured. The resulting data are given in Table 4. It is obvious that a wide variety of carriers may be used. The preference for any one of these is dependent upon other properties besides color value, e.g. wash fastness, physical properties of fiber, heat stability, and light fastness.

50

55

60

65

TABLE 4

| Cationic Dyer                                              |                                            |                                           |                                           |
|------------------------------------------------------------|--------------------------------------------|-------------------------------------------|-------------------------------------------|
| Dye Carrier                                                | Maxilon                                    | Sevron                                    | Sevron                                    |
| Brilliant Orange RA (Color Index Basic Dye Carrier Orange) | Brilliant Red D (Color Index Basic Red 19) | Sevron Blue 5G (Color Index Basic Blue 4) | Sevron Blue 5G (Color Index Basic Blue 4) |
| RA (Color Index Basic Dye Carrier Orange)                  | Brilliant Red D (Color Index Basic Red 19) | Sevron Blue 5G (Color Index Basic Blue 4) | Sevron Blue 5G (Color Index Basic Blue 4) |
| (Color Index Basic Dye Carrier Orange)                     | (Color Index Basic Red 19)                 | Sevron Blue 5G (Color Index Basic Blue 4) | Sevron Blue 5G (Color Index Basic Blue 4) |
| Index Basic Dye Carrier Orange)                            | Index Basic Red 19)                        | Sevron Blue 5G (Color Index Basic Blue 4) | Sevron Blue 5G (Color Index Basic Blue 4) |
| Basic Dye Carrier Orange)                                  | Basic Red 19)                              | Sevron Blue 5G (Color Index Basic Blue 4) | Sevron Blue 5G (Color Index Basic Blue 4) |

|                                                   |        |       |       |
|---------------------------------------------------|--------|-------|-------|
| None                                              | 0.0819 | 0.536 | 0.385 |
| "Cindy" DAC-888                                   | 1.497  | 5.425 | 5.836 |
| Butyl benzoate                                    |        |       |       |
| "Latyl" Carrier A                                 | 1.423  | 4.939 | 6.323 |
| Mixture of benzanilide and dimethyl terephthalate |        |       |       |
| "Carolid"                                         | 1.530  | 6.845 | 7.070 |
| <i>o</i> -Phenylphenol                            |        |       |       |
| "Tanavol"                                         | 1.576  | 5.433 | 6.869 |
| Chlorinated benzene                               |        |       |       |
| "Phenetol" D                                      | 1.700  | 5.704 | 5.794 |
| Mixture of emulsified organic solvents            |        |       |       |
| "Chemo" Carrier KD5W                              | 0.376  | 1.118 | 2.150 |
| Dimethyl phthalate                                |        |       |       |
| "Tanalid" 004                                     | 0.607  | 2.880 | 2.970 |
| <i>p</i> -Phenylphenol                            |        |       |       |
| "Charlab" M-S                                     | 1.187  | 3.810 | 4.837 |
| methyl salicylate                                 |        |       |       |
| Pelargonic Acid                                   | 1.838  | 4.830 | 6.931 |
| Octyl Alcohol                                     | 0.641  | 6.690 | 3.170 |
| Benzyl Alcohol                                    | 0.207  | 1.674 | 8.532 |
| Dimethyl Sulfone                                  | 0.361  | 2.500 | 2.450 |
| Benzoic Acid                                      | 0.410  | 3.090 | 2.620 |
| Dimethyl phthalate                                | 1.519  | 1.325 | 1.486 |
| Hexanol                                           | 1.019  | 2.830 | 7.447 |
| Methyl Salicylate                                 | 1.046  | 5.704 | 5.812 |

## EXAMPLE V

## EFFECT OF TEMPERATURE ON DYEING OF MPD-I

Swatches of MPD-I woven fabric, each weighing 10 g. are introduced into twelve 400 ml. aqueous baths each containing 0.3 g. of one of the dyes indicated in Table 5. Each of the baths also contains 0.1 g. "Merpol" HCS, 1.0 g. zinc thiocyanate (0.25 percent based on weight of water, 10 percent based on weight of fiber), 3.5 g. of "Latyl" Carrier A and 4.0 g. glacial acetic acid. The dye baths are heated to the temperatures indicated in Table 5 and maintained at this temperature for 2 hours. Identical dyeings are performed at 212°F., 230°F., 250°F., and 270°F. (100°C., 110°C., 121°C., and 132°C., respectively). The dyed material is then removed from the baths and rinsed. Then the dyed material is scoured for 30 minutes at 200°F. (93°C.) in 400 ml. of another aqueous bath containing 0.1 g. "Merpol" HCS and 0.1 g. tetrasodium pyrophosphate. The dyed and scoured materials are then rinsed and dried. A series of yellow, red, and blue dyed fabrics is obtained, each having good wet fastness.

The effect of temperature on relative color yield measured by the K/S value is exhibited in the following Table 5.

TABLE 5

| Dye         | Temperature          |                      |                      |                      |
|-------------|----------------------|----------------------|----------------------|----------------------|
|             | 212° F.<br>(100° C.) | 230° F.<br>(110° C.) | 250° F.<br>(121° C.) | 250° F.<br>(132° C.) |
| "Astrazon"  |                      |                      |                      |                      |
| Yellow      | 30                   | 25                   | 100*                 | 90                   |
| 7GLL        |                      |                      |                      |                      |
| "Basacryl"  |                      |                      |                      |                      |
| Red GL      | 35                   | 30                   | 100*                 | 105                  |
| "Calcozine" | 28                   | 30                   | 100*                 | 100                  |
| Acrylic     |                      |                      |                      |                      |
| Blue HP     |                      |                      |                      |                      |

\*Samples dyed at 250° F. (121° C.) were arbitrarily assigned as 100.

## EXAMPLE VI

## DYEING OF MIXED FILAMENT YARN

A mixed filament yarn of 60 denier containing 18 filaments of PACM-12 and 18 filaments of a copolymer derived from bis(4-aminocyclohexyl)methane and a mixture of diacids composed of 90 mole percent dodecanedioic acid and 10 mole percent isophthalic acid is prepared for dyeing in a

package dyer. Twenty-four 1/2-lb. packages are prepared using yarns having 5 turns/inch (2 turns/cm.) Z twist. The yarns are first packaged on collapsible muffs and are then preshrunk by treatment in a steam autoclave at 127°C. for 30 min. The yarn from the muff is then rewound onto 24 perforated steel cylinders. The cylinders are then loaded into a 48 gallon kier with a 5 gallon expansion tank. All subsequent steps, e.g. scouring, dyeing, etc., are conducted at maximum capacity of the kier.

10 The bath:fiber weight ratio is 35:1 for a 12 lb. yarn load. Direction of liquor flow in the kier is changed every three minutes.

The pre-shrunk yarn is scoured with 54.5 g. each of "Merpol" HCS and tetrasodium pyrophosphate for 20 minutes at 180°F. (82°C.) to remove finishes or oils applied during earlier processing. A fresh bath containing 54.5 g. "Merpol" HCS and 1,980 g. citric acid then is prepared at room temperature. To this bath are added 24.5 g., 1.09 g., and 36.5 g. of dye stuffs (1), (2) and (3), respectively, whose formulae are given below:

25



50

After ten minutes, 2,180 g. of a 50 percent aqueous solution of zinc thiocyanate is added [0.5 percent Zn(SCN)<sub>2</sub> based on water, 20 percent based on fiber, 1,760 percent based on dye]. After 10 minutes, the bath is raised to 240°F. (116°C.) at a rate of 3°F./min. (1.67°C./min.). At 160°F., 1,635 g. of butyl benzoate ("Cindy" DAC-472) is added. At 205°F. (96°C.), 60 the kier is closed off from the expansion tank to develop pressure. The dyeing is conducted under pressure for two hrs. at 240°F. (116°C.). Bath temperature is then lowered to 190°F. (88°C.) and the bath discarded. The dyed yarn then is scoured with 54.5 g. each of "Merpol" HCS and tetrasodium pyrophosphate for 20 min. at 140°F. (60°C.) to remove surface dye. The dyed yarns finally are removed from the kier and dried with hot compressed air.

70 The formulation described above provides an attractive, bright fluorescent pink shade on the yarn. Dye wash fastness tests were run on the yarn samples according to the method described in the AATCC Technical Manual, 1968, pages B95 and 96, Test No. 61-1968, Table I, Method IIA, Evaluation Method 8.1. A rating of 4-5 was obtained indicating little or no color change.

## EXAMPLE VII

## EFFECT OF VARIOUS METAL SALTS ON COLOR VALUE K/S

The superiority of zinc thiocyanate as complexing agent over the other metal salts and thiocyanates is illustrated by laboratory piece dyeings using a Vista-matic dyeing apparatus. Dyeings are conducted at bath:fiber ratio of about 60:1 using a jig scoured fabric of plain weave construction containing 120 ends/in. in the warp, and 70 picks/in. in the filling. The yarn in warp and filling is a mixed filament yarn of 60 denier and of the same composition as in Example VI.

Eight 120 ml. baths are prepared at room temperature, each containing 0.02 g. "Merpol" HCS, 2.4 g. citric acid, 0.03 g. dye with formula, as shown below,



and 0.2 g. butyl benzoate ("Cindye" DAC-472). A fabric swatch (2 g.) is introduced into each bath. The effect of various thiocyanates and other salts on dyeability is then determined by adding 0.8 g. of one of the salts shown in Table VI to each dye bath. After 10 minutes, the bath temperature is raised to 212°F. (100°C.) at a rate of 2°F./min. (1.1°C./min.). The dyeing is continued for 2 hours at the boil. The dyed swatches then are scoured in a fresh bath containing 0.02 g. each of "Merpol" HCS and tetrasodium pyrophosphate for 30 min. at 140°F. (60°C.) to remove surface dye. Swatches finally are treated for 2 min. at 325°F. (163°C.) in an oven to remove residual butyl benzoate carrier.

Color value is then determined on each fabric sample and the values shown in Table 6 are obtained. Zinc thiocyanate is shown to be far superior to the other salts, including other thiocyanates, in promoting dyeability of the polyamide fabric with a cationic dye.

TABLE 6

| Complexing Agent     | Color Value, K/S |
|----------------------|------------------|
| Zinc thiocyanate     | 6.3              |
| Calcium thiocyanate  | 1.1              |
| Zinc chloride        | 0.3              |
| Sodium thiocyanate   | 1.5              |
| Ammonium thiocyanate | 1.0              |
| Calcium chloride     | 0.1              |
| Lithium bromide      | 0.4              |
| None                 | 0.3              |

## EXAMPLE VIII

## DYEING WITH VARIOUS CATIONIC DYES

Thirty-nine separate samples of fabric made from the mixed filament yarn described in Example VI are introduced into 39 separate dye baths, each of which contains 2 percent, based on the weight of fibers, of one of the cationic dyes listed

below, and zinc thiocyanate in the amount of 40 percent based on the weight of fibers and 0.1 percent based on the weight of water in the bath. The following standard commercially available cationic dyes were individually used in these baths:

- 5 "Bassacryl" Yellow 5 RL  
 "Bassacryl" Yellow 5 GL  
 "Bassacryl" Yellow 7 GL  
 "Maxilon" Yellow 2 RL  
 "Maxilon" Br. Flavine 10 GFF  
 "Astrazon" Yellow 7 GLL  
 "Maxilon" Br. Yellow 7 GLA  
 "Macilon" Br. Yellow 5 GL  
 "Sevron" Yellow R  
 "Astrazon" Yellow 8 GL  
 "Astrazon" Yellow GRL  
 "Astrazon" Golden Yellow GLD  
 "Astrazon" Orange L  
 "Sevron" Orange G  
 "Maxilon" Br. Orange RA  
 "Astrazon" Orange 3 RL  
 "Astrazon" Pink BL  
 "Astrazon" Pink FBB D/L  
 "Maxilon" Red BL  
 "Sevron" Br. Red 4 G  
 "Sevron" Br. Red D  
 "Astrazon" Pink FG  
 "Sevron" Br. Red B  
 "Sevron" Br. Red BN  
 "Sevron" Br. Red 2 B  
 "Sevron" Br. Red 3 B  
 "Astrazon" Red 6 B  
 "Bassacryl" Violet RL  
 "Maxilon" Br. Green 3 G  
 "Sandocryl" Green BG  
 "Du Pont" Br. Green Crystals  
 "Sevron" Blue 2 G  
 "Maxilon" Blue 5 RL  
 "Sevron" Blue 5 G  
 "Sandocryl" Blue 2 BGLE  
 "Maxilon" Blue 5 G  
 "Sandocryl" Blue B3G  
 "Sevron" Blue EG  
 "Sevron" Blue ER

Each bath is maintained at 90°C. The resulting dyed fabric samples are subjected to wash fastness tests using the AATCC-Wash Fastness Test used in Example VI. None of the 39 dyed fabric samples changed in shade and all had a color value rating of 5.

What is claimed is:

- 50 1. The process for dyeing polyamide fibers comprising contacting said fibers with an aqueous bath containing a cationic dye and zinc thiocyanate at a temperature of at least 90°C., the amount of zinc thiocyanate in the bath being from 1 to 60 percent based on the weight of said fibers and less than 1.5 percent based on the weight of water in the bath.  
 2. The process of claim 1 wherein said polyamide is poly(meta-phenylene isophthalamide).  
 3. The process of claim 2 wherein said bath contains a dye carrier and the temperature of said bath is from 90° to 132°C.  
 60 4. The process of claim 1 wherein said polyamide is poly(methylene-di-1,4-cyclohexylene dodecane diamide).  
 5. The process of claim 4 wherein said bath contains a dye carrier and the temperature of said bath is from 90° to 132°C.

\* \* \* \* \*